

**1****3,718,719****METHOD OF MAKING A COOL BURNING  
GUN PROPELLANT**

Leslie R. Olsen, Barbados, West Indies, assignor to the United States of America as represented by the Secretary of the Navy

No Drawing. Filed Jan. 27, 1971, Ser. No. 110,330

Int. Cl. C06b 21/02

U.S. Cl. 264—3 B

4 Claims

**ABSTRACT OF THE DISCLOSURE**

A cool burning single base gun propellant composition comprised of a blend 12.6 percent nitration level nitrocellulose and 11.0 percent nitration level nitrocellulose in sufficient quantities to provide an average nitration level of 12 percent and a solvent method for the manufacture of said propellant composition wherein a single solvent ratio of ether and alcohol are employed in the colloidization process.

**BACKGROUND OF THE INVENTION**

This invention relates generally to propellants and more particularly to gun propellant compositions and method of their manufacture.

It has been known for some time, that gun wear, i.e., the erosion of the interior of the gun barrel, is caused chiefly by two factors; high temperature of the gases formed upon ignition of the propellant composition and the corrosive effect of these gases upon the metal of the barrel.

Prior attempts to provide gun propellant compositions which minimize these causes of gun wear have been somewhat successful. However, they have not been particularly economical and, on occasion, have created other undesirable side effects due to the addition of ingredients which upon ignition yield gases of discomforting odors.

Other attempts to provide less erosive cool burning gun propellants i.e., possess low flame temperature, also have been advanced. These also have been somewhat uneconomical and have created other problems such as the deposition of large quantities of carbon in the gun barrel which through cumulative effects renders the gun inoperative.

Moreover, recent efforts have been made to utilize the large quantities of obsolete nitrocellulose propellants in stock to avoid the large economic loss that would be incurred by their non-use. Accordingly, a need exists for a cool burning gun propellant employing this unused nitrocellulose.

**SUMMARY OF THE INVENTION**

Accordingly, one object of this invention is to provide a new gun propellant composition and method for its manufacture.

Another object of the present invention is to provide a cool burning gun propellant composition.

Still another object of the instant invention is to provide an economical cool burning gun propellant composition.

Another object of the present invention is to provide an economical cool burning gun propellant composition which may utilize reclaimed nitrocellulose.

Still another object of this invention is to provide a method for the manufacture of a new gun propellant composition which is less tedious and expensive than past processes.

These and other objects are accomplished by providing a single base gun propellant composition comprised of two nitrocellulose grades, one being reclaimed (re-ground) 12.6 percent nitrogen nitrocellulose and the other

**2**

being 11.0 percent nitrogen virgin nitrocellulose. Moreover, the objects of this invention are further accomplished by a method of manufacture of the present gun propellant compositions comprising a solvent process wherein a single solvent ratio of a mixed solvent is capable of forming a homogenous colloid of both of these nitrocellulose grades.

**DESCRIPTION OF THE PREFERRED  
EMBODIMENTS**

10

The gun propellant compositions of the instant invention are comprised of an admixture of 12.6 percent nitrogen nitrocellulose and low grade nitrocellulose of an 11.0 percent nitrogen content. The 12.6 percent nitrogen nitrocellulose may be either virgin nitrocellulose or preferably, for economical purposes, reclaimed nitrocellulose. The processes of reclaiming and reworking obsolete nitrocellulose propellants are conventional and well within the knowledge of one skilled in the art. Generally, the old nitrocellulose is ground and pulverized and since the potential energy level remains essentially unaltered, the whole process is basically merely a regrinding procedure.

However, whichever of the 12.6 percent nitrogen nitrocellulose is utilized, it and the virgin 11.0 percent nitrogen nitrocellulose are blended together in sufficient quantities to provide a gun propellant with an average nitration level of nitrocellulose of 12 percent.

Thus, according to the instant invention, the unexpected discovery was made of a cool burning and less erosive gun propellant having an average nitration level of 12 percent by weight employing nitrocelluloses of nitration levels differing as much as 1.6 percent, and wherein one of these nitrocellulose grades may be reclaimed nitrocellulose, which is at least comparable in ballistic performance and chemical stability to a propellant made from one nitration level of nitrocellulose of 12 percent.

The gun propellant compositions made in accordance with the present invention generally contain a large percentage of nitrocellulose, i.e., from about 87 to about 95 percent by weight. Of course, other ingredients normally employed in compositions of this nature also may be included in relatively minor amounts. For example, inorganic salts such as potassium sulfate and/or potassium nitrate may be incorporated as flash suppressants from about 1 to 3 percent by weight. Stabilizers and coolants, such as ethyl centralite and butyl stearate, may be used in amounts of about 1 percent for the centralite to amounts of from about 2.5 to about 6 percent of the butyl stearate. Additionally, lubricants, such as basic lead carbonate, may be also included in about 1 percent by weight quantities of the total composition.

The process employed in the manufacture of the gun propellant compositions of the instant invention is begun following conventional steps for the preparation of nitrocellulose gun propellant compositions. That is, in the instant process, as in the prior art processes, the nitrocellulose is dehydrated, if water wet, or wrung of excess alcohol, if alcohol wet, down to a known level. Unlike prior art processes, the present process employs nitrocelluloses differing in nitration levels to the extent of about 1.6 percent in quantities sufficient to provide a final blend of nitrocellulose characterized by an average nitration level of about 12 percent.

The differing nitration level nitrocelluloses are blended and mixed together with some of the other dry propellant ingredients to be used, such as the potassium sulfate and the basic lead carbonate in a conventional propellant mixer. Traditionally, ethyl centralite and butyl stearate are not added dry but rather in ether solution for more optimized mixing.

At this point, the nitrocellulose mixture is colloided employing a mixed ether/alcohol solvent. It is intended that ether and alcohols refer to diethyl ether and ethyl alcohol.

It has been found in the present process that a single solvent ratio of from about 30:70 to about 35:65 parts by weight of ether and alcohol, respectively, is sufficient to form a good colloidal mixture of the 11.0 percent nitration nitrocellulose and the 12.6 percent nitration nitrocellulose. Preferably a 32:68 parts by weight ether/alcohol ratio is used.

In prior art process of manufacturing propellant compositions using different nitration level nitrocelluloses, each nitrocellulose requires a separate colloiding process with a different solvent ratio thereby adding to the tediousness and expense of the process.

The quantity of solvent employed in the instant process, i.e., solvent level, is generally from about 80 to about 90 percent by weight of the total composition. Preferably about an 85 percent solvent level is employed. Any of the residual alcohol already present in the nitrocellulose and/or ether employed in the addition of other ingredients to the composition are taken into consideration in the calculation of the quantity level and ratio of the mixed alcohol/ether solvent. Furthermore, adjustments of the solvent level and ratio must be commensurate with volatile losses during the mixing cycles of the composition.

After colloidalization is complete, the remaining steps of the process follow conventional lines. Thus, the propellant compositions is removed from the mixer and pressed into cylindrical blocks. These blocks of propellant are then strained into strands to remove any uncolloided particles and blocked again. The blocks are extruded into strands, the strands are cut and then dried to a minimum or desired level of volatile content. In the context of this invention, volatiles is intended to mean such things as water, alcohol and ether.

The mixing process of the instant invention may be performed at various temperatures depending on processing considerations as is the case with conventional procedures for mixing propellants of this nature. For example, a temperature of 75° F. has been found to be desirable.

The general nature of the invention having been set forth, the following example is presented as a specific illustration thereof. It will be understood that the invention is not limited to this example but is susceptible of different modifications that will be readily recognized by one of ordinary skill in the art.

#### EXAMPLE

A 93 percent by weight nitrocellulose gun propellant having an average nitration level of about 12 percent was made according to the following procedure: about 162 pounds (dry weight) of reground (reclaimed) 12.6 percent nitration level nitrocellulose, about 98 pounds (dry weight) of virgin 11.0 percent nitration level nitrocellulose, 2 pounds of basic lead carbonate and 4 pounds of potassium sulfate were dry mixed in a conventional horizontal propellant mixer. 9 pounds of butyl stearate and 2 pounds of ethyl centralite were dissolved in 74.84 pounds of diethyl ether and were added to the nitrocellulose mixture in conjunction with about 152 pounds of ethyl alcohol. The total mix was agitated, at about 75° F., until a homogenous colloid was obtained and subsequently removed from the mixer. This mixture was then processed in a conventional manner, i.e., the mixture was pressed into cylindrical blocks in a 12 inch vertical press. It was then strained, reblocked and extruded in the same press and cut and dried.

The solvent level used in the exemplary process was 81 percent wherein the 12.6 percent nitration level nitrocellulose was initially alcohol wet and had a total volatiles content of about 23 percent by weight, while the 11.0 percent nitration level nitrocellulose also was initially alcohol wet and had a total volatiles content of about 22 percent by weight. The solvent ratio of ether to alcohol was 33:67 parts by weight and the total volatiles content of the final propellant composition was about 3.27 percent by weight.

10 The gun propellant compositions of this invention, as exemplified by the example, have a nominal adiabatic flame temperature in the range of from about 2000° K. to about 2200° K.

15 The composition of the example was manufactured in prototype lots of about 10,000 pounds and were evaluated by extensive gun firing tests in 5-inch/54-caliber guns. The average muzzle velocity obtained was about 2650 feet per second and the average breach internal pressure within the gun was about 20.2 tons per square inch.

20 Obviously, numerous modifications and variations of the present invention are possible in the light of the above teachings. It is therefore to be understood that within the scope of the appended claims the invention may be practiced otherwise than as specifically described herein.

25 What is claimed and desired to be secured by Letters Patent of the United States is:

30 1. A process for the manufacture of a single base gun propellant composition comprising the steps of:

(a) mixing a sufficient quantity of 12.6 percent nitration level nitrocellulose with a sufficient quantity of 11.0 percent nitration level nitrocellulose to provide a nitrocellulose mixture of an average nitration level of about 12 percent,

35 (b) adding to and mixing with the mixture of step (a) a solvent mixture consisting essentially of a mixture of diethyl ether and ethyl alcohol for a sufficient time to form a colloidal mixture therewith, wherein said solvent mixture is added in a sufficient quantity to provide a solvent level of from about 80 to about 90 percent by weight of the total composition and wherein said solvent mixture is in a ratio of from about 30:70 to about 35:65 parts by weight of diethyl ether to ethyl alcohol, and

40 (c) blocking, extruding and drying the product of step (b).

45 2. The process of claim 1 wherein said solvent mixture is added in a sufficient quantity to provide a solvent level of about 85 percent by weight of the total composition and wherein said solvent mixture is in a ratio of about 32:68 parts by weight of diethyl ether to ethyl alcohol.

50 3. The process of claim 1 wherein said 12.6 percent nitration level nitrocellulose is reclaimed nitrocellulose.

55 4. The process of claim 2 wherein said 12.6 percent nitration level nitrocellulose is reclaimed nitrocellulose.

#### References Cited

##### UNITED STATES PATENTS

|    |           |         |                      |           |
|----|-----------|---------|----------------------|-----------|
| 60 | 3,014,246 | 12/1961 | Cook et al. _____    | 264—3 BX  |
|    | 3,116,190 | 12/1963 | Zihlman et al. _____ | 149—100   |
|    | 3,317,361 | 5/1967  | Hopper et al. _____  | 149—96 X  |
|    | 3,473,982 | 10/1969 | Herzog et al. _____  | 149—100 X |

65 BENJAMIN R. PADGETT, Primary Examiner

S. J. LECHERT, Jr., Assistant Examiner

70 U.S. CL. X.R.

149—94, 96, 100